

Nov. 21, 1939.

R. STRIBECK

2,180,779

ETCHED SPARKING PLUG

Filed June 18, 1938



Inventor  
Richard Stribeck  
by Roy F. Steward  
his attorney

## UNITED STATES PATENT OFFICE

2,180,779

## ETCHED SPARKING PLUG

Richard Stribeck, Stuttgart, Germany, assignor  
to Robert Bosch Gesellschaft mit beschränkter  
Haftung, Stuttgart, Germany

Application June 18, 1938, Serial No. 214,557  
In Germany July 9, 1937

8 Claims. (Cl. 123—169)

During the operation of a sparking plug in an internal combustion engine, the temperature which the insulator of the plug takes up fluctuates through several hundred degrees Celsius and generally lies between 300 and 900° C. These temperature differences occur in that part of the insulator which projects furthest into the combustion chamber and, under certain working conditions of the engine, they take place within a few seconds. The stability of the insulator of the sparking plug to temperature change is not, however, tested only by the temperature variation occurring at a particular determined point of the insulator, but also by the degree of the temperature decrease in the interior and along the surface of the insulator. Especially at the surface of the insulator in the neighbourhood of the points situated at the highest temperature, or on the collar of the insulator, at which the heat is conducted away from the metal body of the plug, there occur high temperature drops which endanger the stability of the insulator by giving rise to the formation of cracks and flaws.

Hitherto efforts have been made to improve the stability of the sparking plug insulator to temperature change by using special ceramic masses for the manufacture of the said plug, or, by constructional formation of the plug, to cause a decrease of the thermal stresses connected with use. Despite the good result of the steps undertaken in these directions, the occurrence of cracks in the insulator is still noticed under unfavourable circumstances, especially in plugs which are used in engines which are submitted to sharply changing stresses, and are often submitted to the maximum stress.

It has also been proposed to roughen ceramic insulators or insulators consisting of glass or glazed masses, for the purpose of increasing the resisting power relative to temperature fluctuations. However, it has been found that roughening the surface does not increase the stability of sparking plug insulators to temperature change, but that a surface made rough by, for instance, sand jets merely conceals the cracks and flaws which have arisen owing to thermal stress, or makes them less easily visible. The known etching of the insulators by means of acids or lyes also does not lead to an increase of the stability to temperature change when the insulators consist of a mass which is attacked throughout by the etching medium, which is the case for instance, in sparking plug insulators made from sillimanite ( $Al_2O_3 \cdot SiO_2$ ) and steatite insulators.

Now it has been found that such plug insulators

consisting of a burnt ceramic mass which contain both components which are not attacked or not substantially attacked by the etching medium, and also components which are dissolved by the etching medium can be substantially improved as regards stability to temperature change by a superficial etching. Insulators of this kind are, for instance, such as contain as the material which is not soluble in the etching medium, corundum, spinel, (e. g.  $MgO \cdot Al_2O_3$ ) or silicon carbide and which, for the remainder, consist of a ceramic mass which is soluble in the etching medium.

The etching medium should be selected to correspond to the particular composition of the insulator. Generally, hydrofluoric acid is suitable but salts or lyes, such as sodium carbonate or caustic potash, may also be used in a fused condition as the etching medium.

A considerable improvement in stability to temperature change is experienced especially by the insulators which contain more than 30% corundum and contain in addition to corundum a burnt ceramic mass serving as the combining agent for the corundum, by etching by means of hydrofluoric acid. Of the components of an insulator of this kind, the corundum is substantially insoluble in hydrofluoric acid, while the binding agent is soluble. The etching dissolves the ceramic binding agent of the surface layer and leaves on the surface of the insulator corundum crystals which are connected with each other in the manner of a skeleton.

The temperature and concentration of the hydrofluoric acid and the duration of the etching treatment should be adapted to the particular circumstances, especially to the solubility of the component of the plug insulator which is soluble in hydrofluoric acid. Generally, hydrofluoric acid at any temperature up to 100° C. can be used in a concentration of 20—40%  $H_2F_2$ , and the duration of treatment can amount to a few minutes up to two hours. By way of example, the stability to temperature change of an insulator which contains about 70% corundum and the remainder ceramic binding agent, was substantially improved by immersion for a quarter of an hour in hydrofluoric acid containing 40%  $H_2F_2$  and heated to 40° C. The depth of the etching can amount to up to about 0.5 mm.

The process according to the invention is appropriately carried out in such a way that only those parts of the plug insulator which are thermally highly stressed are superficially etched. By means of the drawing, there is explained by

way of example what is to be understood by the thermally highly stressed parts of the plug insulator. In the drawing, there is shown partly in section a sparking plug consisting of the plug insulator *a*, the lug body *b* and the middle electrode *c*. The plug insulator is thermally stressed from the foot *x* to the collar *y*. At the foot *x* there occur the highest temperatures and greatest temperature fluctuations, and at the collar *y*, where the heat of the plug insulator is carried off from the plug body *b* by means of the packing ring *d*, there exists during the operation of the plug, a permanent sharp temperature drop. By etching treatment of those parts at which cracks usually occur, the stability to temperature change can be improved and the formation of cracks can be avoided.

The presence of a glaze makes it more difficult to carry out the process according to the invention, since the glaze layer must be completely dissolved away before the etching medium can act in the desired manner. For this reason it is recommended to use only such plug insulators as are not glazed at the points to be etched. It will generally be appropriate to submit the foot of the plug upwards to the middle of the plug collar—in the plug insulator in the drawing, the plug foot *x* upwards to the dotted line—to the etching treatment. Especially plug insulators containing corundum in a larger quantity than 30% have proved outstandingly stable to temperature change, when the plug foot, including the lower part of the plug collar, has been superficially etched by means of hydrofluoric acid.

I declare that what I claim is:

1. A process for improving the stability to temperature change of sparking plug insulators consisting of a burnt ceramic mass of insoluble and soluble components, which comprises superficially etching said insulators by contacting them with an etching medium which attacks the soluble components but which does not substantially attack the insoluble components.

2. A process for improving the stability to temperature change of sparking plug insulators consisting of a burnt ceramic mass of insoluble and soluble components, in which the sparking plug insulators are etched superficially by hydrofluoric acid.

3. A process for improving the stability to temperature change of sparking plug insulators consisting of a burnt ceramic mass of insoluble and soluble components, the plug insulators containing more than 30% by weight of corundum, which comprises superficially etching said insulators by contacting them with an etching medium which attacks the soluble components but which does not substantially attack the insoluble components. 5

4. A process for improving the stability to temperature change of sparking plug insulators consisting of a burnt ceramic mass of insoluble and soluble components, in which those parts of the plug insulators which are thermally highly stressed are etched superficially by hydrofluoric 10 15 acid.

5. A process for improving the stability to temperature change of unglazed sparking plug insulators consisting of a burnt ceramic mass of insoluble and soluble components, which comprises 20 superficially etching said insulators by contacting them with an etching medium which attacks the soluble components but which does not substantially attack the insoluble components.

6. A sparking plug insulator which consists of 25 a burnt ceramic mass containing 30% by weight at least of corundum, in which the foot of the plug insulator has been etched by means of hydrofluoric acid.

7. A process for improving the stability to temperature change of sparking plug insulators consisting of a burnt mass of insoluble and soluble components comprising about 70% corundum and the remainder ceramic binding agent which comprises contacting said insulators with hydrofluoric acid until they are superficially etched. 35

8. A process for improving the stability to temperature change of sparking plug insulators consisting of a burnt mass of insoluble and soluble components comprising about 70% corundum and the remainder ceramic binding agent which comprises immersing said insulators in hydrofluoric acid containing about 40%  $H_2F_2$  and heated to about 40° C. until they are etched to an amount up to 0.5 mm. 40 45

RICHARD STRIBECK.